

(No Model.)

J. MORRIS.

COMBUSTIBLE VAPORIZING CASE.

No. 399,230.

Patented Mar. 5, 1889.



Witnesses:

C. J. Hedrick

H. O. Tracy

Inventor:

John Morris  
by A. Hobbs  
his attorney.

# UNITED STATES PATENT OFFICE.

JOHN MORRIS, OF SHIRLEY COTTAGE, SOUTH VIEW, BASINGSTOKE, ENGLAND, ASSIGNOR TO THE CHEMICAL CARBON COMPANY, (LIMITED,) OF SAME PLACE.

## COMBUSTIBLE VAPORIZING-CASE.

SPECIFICATION forming part of Letters Patent No. 399,230, dated March 5, 1889.

Application filed June 20, 1888. Serial No. 277,649. (No model.) Patented in England March 3, 1885, No. 2,786.

*To all whom it may concern:*

Be it known that I, JOHN MORRIS, chemist, a subject of the Queen of Great Britain, and residing at Shirley Cottage, South View, Basingstoke, England, have invented certain improvements in carbon cones and cases for distributing medicinal matters, disinfectants, fumigants, perfumes, and the like, (for which I have obtained a patent in Great Britain, No. 2,786, dated the 3d day of March, 1885,) of which the following is a specification.

Very-finely-powdered carbon is intimately mixed with levigated fused nitrate of potash in varying proportions with or without the addition of gum. These ingredients are then wetted and subjected to a further incorporation in a rolling and kneading mill of such power as will permit of a heavy pressure being imposed upon the mixed materials, such as will render the resultant mass homogeneous and dense in character. The proportions of the fused nitrate of potash vary from the maximum of twenty-five per centum of the quantities of the carbon used downward to five per centum, or less, according to the rate of combustion required. The carbon may be first treated with acids or the like for the removal of certain mineral constituents and the destruction of certain impurities. At option I employ definite proportions of silicates or finely-divided glass for tempering the mixed mass of carbon and nitrate of potash with (or without) gum.

The tempering materials are used in varying proportions, usually being five per centum of the whole weight of the materials operated upon. After a thorough incorporation in the rolling and kneading mill the mass is at once worked up into cones or cases. These cones or cases are made in the desired forms, which may be effected by means of polished gunmetal molds of the following description:

A central solid core of metal is provided, with a highly-polished surface, either cone-shaped or of such other shape as will form the interior space of the desired cone or case, and a corresponding hollow mold of the same metal equally polished on its internal surface, whose inside diameter exceeds in any part

the diameter of the interior solid cone or otherwise-shaped core, part for part. A portion of the mixed carbonaceous mass is then placed within the hollow mold, and is by any suitable mechanical arrangement subjected to heavy pressure over the solid internal core of metal, a hollow cone or case being thus produced whose walls are equal. These cones and cases are then removed from the molds and are at once subjected to a dry heat of not less than 220° Fahrenheit for a space of from five to fifteen minutes, having regard to their varying sizes and quantities of material. The temperature is then lowered to from 160° to 180° Fahrenheit, at which they are dried off. They are afterward provided with bases made of fine clay, aluminous, or any other material of such nature, such as proves incombustible up to and inclusive of a temperature equaling 500° Fahrenheit, for the purpose of mitigating the effects of the heat given off in the act of combustion. The apexes or tops of these cones or cases may be tipped with any quickly-lighting material to accelerate their combustion.

The materials which these cones and cases are to convert into vapor are placed within the cones and cases.

In the accompanying drawing, which forms part of this specification, A represents the carbon cone, B a glass receptacle inside the carbon cone and containing the material to be vaporized, and C represents the incombustible support for the carbon cone.

It is important to notice that by increasing or decreasing the wall thicknesses of the cones and cases I am able to develop and command a range of heat more quickly and effectually for the ends in view than by any other method, the portability of the means for so doing being duly regarded.

By providing a case which is incombustible at a comparatively high range of temperature I obviate to a great extent injuries that may be caused by the combustion of carbonaceous matters for the above purposes.

I claim—

1. The within-described cone or case for dissipating active materials in a state of vapor,

said cone or case being composed, essentially, of carbon combined or mixed with nitrate of potash, substantially as set forth.

2. A combustible cone or case for the purpose specified, composed of carbon and levigated fused nitrate of potash, and provided with an incombustible support or base, substantially as described.

In testimony whereof I have signed my name to this specification in the presence of two subscribing witnesses.

JOHN MORRIS.

Witnesses:

CHAS. MILLS,

EDWD. GEO. DAVIES.

*Both of 47 Lincoln's Inn Fields, London.*